

3,458,296

## FUEL OIL COMPOSITION

Gordon G. Knapp, Southfield, and Joseph P. Kleiman, Royal Oak, Mich., assignors to Ethyl Corporation, New York, N.Y., a corporation of Virginia  
No Drawing. Filed Dec. 7, 1966, Ser. No. 599,713

Int. Cl. C10l 1/18; C06b 15/00

U.S. Cl. 44-66

7 Claims

## ABSTRACT OF THE DISCLOSURE

A fuel oil composition having improved cold flow containing from about 0.04 to about 0.5 percent by weight of an ester of palmitic acid and an anhydroalkitol. An anhydroalkitol is a cyclic ether product obtained from intramolecular dehydration of polyhydroxy alcohols having 5 or 6 carbon atoms. The palmitates of anhydro-sorbitol are preferred esters.

## Background of the invention

Residual and distillate petroleum hydrocarbons are used as fuels in various applications. They are used as diesel fuels, jet fuels, home heating fuel, turbine fuels, rocket fuels, and in similar combustion systems. It is recognized that the fluidity of fuel oils in general is reduced as they are cooled. Additives which reduce the tendency of these fuels to become more viscous at low temperatures are available and are called pour point depressants. Another phenomenon which occurs when these fuels are cooled is that orifices and other narrow openings through which the fuel passes tend to become plugged. This occurs even when the fuel oil contains pour point depressants adequate to maintain proper viscosity at low temperatures. This latter characteristic of fuel oils, that is, their ability to flow through narrow orifices at low temperatures is referred to as cold flow.

In view of this need to overcome orifice plugging at low temperatures, additives which function as cold flow improvers in fuel oils are of substantial importance. As stated above, this invention comprises the discovery that certain esters of palmitic acid and anhydroalkitols are effective cold flow improvers in hydrocarbon fuel oils.

## Summary of the invention

This invention relates to hydrocarbon fuel oil compositions having improved cold flow. It more particularly relates to fuel oil compositions containing esters of palmitic acid and an anhydroalkitol, said alkitol having from 5 to 7 carbon atoms. A preferred embodiment relates to a method for improving the cold flow characteristics of a fuel oil by adding thereto a small amount of an ester of palmitic acid and an anhydrosorbitol.

It is an object of this invention to provide a fuel oil having improved cold flow properties. It is a further object of this invention to provide a fuel oil containing a small amount of an ester of palmitic acid and a C<sub>4</sub> to C<sub>7</sub> anhydroalkitol sufficient to improve the cold flow characteristics of the fuel. Still another object of this invention is to provide a method for improving the cold flow characteristics of a fuel oil by adding thereto a small quantity of an ester of palmitic acid and a C<sub>5</sub> to C<sub>7</sub> anhydroalkitol. These and other objects of the invention will be made clear from the description and claims which follow.

## Description of the preferred embodiments

An embodiment of this invention is a fuel oil having improved cold flow characteristics containing from 0.04 to about 0.5 percent by weight of an ester of palmitic acid and an anhydroalkitol, said anhydroalkitol having 5 to 7 carbon atoms. A preferred embodiment of this invention

is the fuel oil described above wherein the ester is present at a concentration of about 0.06 to about 0.1 percent by weight. A more preferred embodiment of this invention is the fuel oil described above wherein the ester is selected from the group consisting of sorbitan monopalmitate, sorbide monopalmitate, sorbitan dipalmitate, sorbide dipalmitate, and mixtures thereof. Still more preferred embodiments of this invention are fuel oils described above wherein the ester is sorbitan palmitate; and fuel oils described above wherein the ester is sorbitan dipalmitate. A most preferred embodiment of this invention is a fuel oil as described above wherein the ester is sorbide monopalmitate or sorbide dipalmitate.

The fuels which are used in the compositions of this invention are petroleum hydrocarbons. They may be distillate fuels, residual fuels or blends of these two types. The distillate fuels are fractionation cuts from the distillation of either crude oil or the products from a cracking process. Cracked distillates are usually blended with straight run distillates before using. Kerosene is a typical distillate fuel. A residual fuel oil is the viscous product left after the more volatile fractions have been distilled or topped from the crude oil. It is the least expensive of the fuels obtainable from petroleum. It is used alone as well as in blends with the lower boiling distillate fuel fractions.

These fuels are also characterized by their boiling point range. In general, the useful fuels have a boiling point ranging from about 100° F. to about 1,000° F. The boiling point on most commonly used fuels ranges from about 200° F. to about 800° F. Useful fuels include diesel fuel oil grade DF-A, DF-1, DF-2; domestic fuel oils Nos. 1, 2, 3, 4 and 5; jet fuels such as JP-1, JP-4, JP-5, and the like.

The cold flow improver compounds which are used in the fuel compositions in the present invention are esters of palmitic acid and C<sub>4</sub> to C<sub>7</sub> anhydroalkitols. An anhydroalkitol is an intramolecular dehydrogenation product of an alkitol. The term alkitol means a polyhydric alcohol having at least 4 carbon atoms and at least 4 hydroxyl groups. Examples of suitable alkitalols are mannitol, dulcitol, xylitol, and the like. A most preferred alkitol is sorbitol.

The alkitalols are readily dehydrated to form cyclic ether type compounds. When one molecule of water is lost from an alkitol by intramolecular dehydration, a polyhydric monocyclic ether is produced. The generic name for such a compound is an alkitan. When two molecules of water are removed from an alkitol by intra-molecular dehydration, a polyhydric dicyclic ether is produced. The term alkide is applied to this product. Thus, for example, if dulcitol were dehydrated, the product obtained on removing one molecule of water would be termed dulcitan; if two molecules of water were removed, the product would be termed dulcide.

Anhydroalkitols which are preferred are the products obtained by intramolecular dehydration of sorbitol. When one molecule of water is thus removed, the product is sorbitan; when two molecules of water are thus removed, the product is sorbite.

Esters which are suitable for the purpose of this invention are those obtained by reacting the alkitalols and alkides described above with palmitic acid. Palmitic acid is a 16 carbon saturated monocarboxylic acid. It is commonly obtained by hydrolyzing palm oil and separating it from the mixed product; the acid can also be made synthetically, as for example, by carbonylating a suitable olefin in the presence of water.

The esters which are useful in the present invention include the monoesters, the diesters and mixtures thereof. Monoesters are those in which one hydroxyl group in

the alkitan or alkide is esterified. Examples of useful monoesters are dulcitan monopalmitate, mannide monopalmitate, adonitan monopalmitate, and the like. Preferred monoesters are sorbide monopalmitate and sorbitan monopalmitate.

Diesters are obtained when two hydroxyl groups are esterified. Useful diesters are manitan dipalmitate, xylitan dipalmitate and dulcide dipalmitate. Diesters which are preferred are sorbitan dipalmitate and sorbide dipalmitate.

Mixtures of these alkide and alkitan esters are also useful. Thus, for example, mixtures of manitan mono- and dipalmitate; sorbide monopalmitate and dipalmitate; dulcitan monopalmitate and dulcide monopalmitate; sorbide dipalmitate and sorbitan dipalmitate; mannide monopalmitate and sorbide monopalmitate, and the like are useful in the compositions of this invention.

These ester mixtures may also include the alkide and alkitan esters of other fatty acids. Thus, for example, sorbide or sorbitan may be esterified with the mixed acids obtained from palm oil. A typical composition of fatty acids obtained from palm oil is 42½ percent palmitic acid, 43 percent oleic acid, with the remainder being myristic, stearic and linoleic acid. Using this mixture of acids, the sorbitan or sorbide ester product will contain analogous quantities of the various esters, that is, palmitates, myristates, oleates, stearates and linoleates. Such ester mixtures are useful in the practice of this invention. When making up the fuel oil compositions, sufficient quantities of the mixed ester would be used in order that the concentration of palmitate esters is within the weight range disclosed above. The mixed acids may also be those obtained from commercial synthesis processes such as from Ziegler catalyzed chain growth procedures. On the other hand, the mixed acids may be purposely blended for economic reasons and then used to esterify alkitan and alkides. In general then, mixed esters containing other carboxylic alkyl residues besides palmitate may be used in the practice of this invention.

The anhydroalkitol esters which are used in the present invention are well known compounds. Methods for their preparation are given in the literature. Procedures for their preparation are presented in U.S. 2,322,820 and U.S. 2,398,193. The procedures described in these patents are conveniently used to make esters used in the present invention.

The following examples illustrate typical ester preparations. All parts are by weight unless otherwise specified.

#### Example 1

A mixture of 52 parts of sorbitol syrup and 102.6 parts of palmitic acid and about 0.1 part of 85 percent phosphoric acid were heated to 200° F. in a suitable vessel with stirring in a nitrogen atmosphere. The temperature of the mixture was maintained between 200° and 250° C. until no more water came off. (Small amounts of toluene were added to the reaction mixture to prevent palmitic acid from clogging the condenser and to azeotrope the water.) When all of the water was removed, the reaction mixture was cooled. The product was dissolved in petroleum ether and recrystallized. The yield was 120 parts of sorbide dipalmitate.

#### Example 2

To a reaction vessel fitted with condenser, inlet tube and stirrer are added 260 parts of sorbitol syrup (70 percent sorbitol), about 2 parts of sodium hydroxide, and 256 parts of palmitic acid. The mixture is stirred and heated at 220° to 240° C. Water of reaction is constantly being removed. The dehydration and esterification are complete after 4 hours. The product obtained is sorbitan monopalmitate.

The quantity of ester which is used to prepare the improved fuel compositions of the present invention may be from 0.04 to about 0.5 percent by weight of the

fuel oil. The preferred range is 0.05 to about 0.1 percent by weight. The optimum amount of ester which is added to the fuel oil will depend to some extent on the nature of the fuel oil and the lowest temperature at which the oil will be used.

The fuel oil compositions of the present invention can be prepared by dissolving the ester additive directly in the fuel. Special equipment is not required and conventional liquid mixing or blending equipment may be used. The ester additive may, on the other hand, be dissolved in a suitable solvent to form an additive concentrate. This additive concentrate may then be used to prepare the fuel oil composition of this invention. The additive concentrate may contain up to 50 percent by weight of the ester additive. In either case, that is whether the ester is added (a) directly to the fuel or (b) as an additive concentrate, the final effective concentration of additive in the fuel oil will be within the ranges disclosed above.

In order to show the unobvious improvement in cold flow in fuel compositions of this invention, the fuel oil compositions were evaluated using the Enjay Fluidity Test. The Enjay Fluidity Test measures the flow characteristics of fuel oils through a narrow orifice. The procedure and test equipment are fully described in Enjay's brochure ELD-48439. The contents of that brochure are incorporated by reference as part of this specification. Briefly, the test involves measuring the amount of fuel oil which flows through an orifice in a given time at a given temperature. The testing device consists of a two-compartment cylinder connected by means of a capillary tube ½ inch long and 2.25 mm. inside diameter. Each chamber is calibrated. Forty milliliters of the fuel oil to be tested are placed in one chamber of the cylinder; the cylinder is capped, inverted so that the fuel will not run into the other chamber, and placed in a bath set at the desired temperature for two hours. At the end of this time, the cylinder is inverted so that the cooled fuel now can run through the capillary tube into the second chamber. The test apparatus is kept in the cooling bath while the fuel is allowed to flow for three minutes. At this point, the amount of fuel which has flowed through is measured. It is reported as percent recovery of total fuel sample used. The higher the percent of fuel which passes through, the better cold-flow the fuel composition has. Thus, for example if 20 ml. of fuel oil flows from the first chamber to the second chamber, the Enjay Fluidity Recovery is 50 percent.

Following are the Enjay Fluidity results obtained in running a series of fuels. The ester additives were prepared using the procedures disclosed above. All the tests were conducted at -25° F.

TABLE I.—ENJAY FLUIDITY

| Fuel No. <sup>1</sup> | Additive               | Weight percent additive | Recovery <sup>2</sup> Percent |
|-----------------------|------------------------|-------------------------|-------------------------------|
| 1                     | None                   |                         | 0                             |
| 2                     | Sorbide Dipalmitate    | 0.10                    | 93                            |
| 3                     | Sorbide Monopalmitate  | 0.10                    | 82.5                          |
| 4                     | do                     | 0.08                    | 71.7                          |
| 5                     | do                     | 0.06                    | 36.2                          |
| 6                     | Sorbitan Monopalmitate | 0.10                    | 59                            |

<sup>1</sup> The base fuel used was Mobil Grade No. 2 fuel oil.

<sup>2</sup> Average of two runs.

The data in Table I clearly indicates the effectiveness of the sorbide and sorbitan palmitate esters as cold flow improvers. The base fuel without any additive would not flow through the capillary tube in the Enjay test apparatus. Addition of from 0.06 to 0.1% by weight of either the sorbide or sorbitan palmitate improves this cold flow characteristic of the fuel to the point where up to 93% of the fuel did flow through the capillary tube at -25° F.

Comparable improvement in cold flow is obtained when analogous anhydro mannitol, anhydrolulcitol, anhydroxylitol esters and the like are used in place of the sorbide or sorbitan palmitates.

A series of fuel compositions were also run to show the criticality of the  $C_{16}$  alkyl moiety in the esters of this invention. Again all tests were made at  $-25^{\circ}$  F. using the Enjay Fluidity Test described above. The data are presented in Table II below.

TABLE II

| Fuel containing 1—     | Alkyl portion of ester | Enjay fluidity recovery, percent |
|------------------------|------------------------|----------------------------------|
| Sorbide dipalmitate    | $C_{16}$               | 93                               |
| Sorbide dioleate       | $C_{18}$               | 13                               |
| Sorbitan Monolaurate   | $C_{12}$               | 1                                |
| Sorbitan Monomyristate | $C_{14}$               | 13                               |
| Sorbitan Monopalmitate | $C_{16}$               | 59                               |
| Sorbitan Monostearate  | $C_{18}$               | 5                                |
| Sorbitan Monolinoleate | $C_{18}$               | 11                               |
| Sorbide Monolaurate    | $C_{12}$               | 3                                |
| Sorbide Monomyristate  | $C_{14}$               | 19                               |
| Sorbide Monopalmitate  | $C_{16}$               | 83                               |
| Sorbide Monostearate   | $C_{18}$               | 5                                |
| Sorbide Monolinoleate  | $C_{18}$               | 15                               |

<sup>1</sup> Base fuel is the same as that used in fuels of Table I; concentration of additive in each case is 0.1 weight percent.

The data in Table II clearly illustrates the unexpected superiority as cold flow improvers of the  $C_{16}$  alkide and alkanoate esters over homologous  $C_{12}$ ,  $C_{14}$  and  $C_{18}$  esters. This increased potency is surprising and wholly unexpected. Thus, when sorbide monopalmitate is added to fuel oil, 83 percent recovery at  $-25^{\circ}$  F. is effected. Using the same amount of the analogous  $C_{14}$  or  $C_{16}$  ester, that is, the monomyristate or monostearate, there is a marked decrease in cold flow activity as indicated by the lower percent recovery. It is readily apparent then that the alkyl portion of the anhydroalkanoate esters useful in this invention must have 16 carbon atoms in order that the fuel oil compositions containing the esters have substantially improved cold flow characteristics.

In addition to the anhydroalkanoate esters, the fuel oils of the present invention may contain other additives. Thus, the fuel oil may contain combustion improvers such as amyl nitrate, acetoneperoxide, and the like; smoke reducers such as overbased calcium sulfonates, methylcyclopentadienyl manganese tricarbonyl, and the like; corrosion inhibitors such as linoleic acid dimer and the like; antioxidants such as 2,6-di-tert-butylphenol,  $N,N'$ -di-sec-butyl-p-phenylene diamine and the like; metal deactivators such as  $N,N'$ -disalicylidine,

1,2-propane diamine and the like. Any or all of these types of additives may be present in the fuel oil provided that they do not inhibit the cold flow activity of the anhydroalkanoate esters.

The compositions of our invention are fully described in the disclosure presented above. The specification includes data which points out and confirms the unobvious and unexpected nature of this invention. It is not intended that the invention be limited except within the lawful scope of the following claims.

We claim:

1. A fuel oil having improved cold flow characteristics containing from 0.04 to about 0.5 percent by weight of an ester of palmitic acid and an anhydroalkanoate, said anhydroalkanoate having from 5 to 7 carbon atoms.

2. The fuel oil of claim 1 wherein said fuel oil contains from about 0.06 to about 0.1 percent by weight of said ester.

3. The fuel oil of claim 1 wherein the ester is selected from the group consisting of sorbitan monopalmitate, sorbitan dipalmitate, sorbide monopalmitate, sorbide dipalmitate and mixtures thereof.

4. The fuel oil of claim 3 wherein the ester is sorbitan palmitate.

5. The fuel oil of claim 3 wherein the ester is sorbitan dipalmitate.

6. The fuel oil of claim 3 wherein the ester is sorbide monopalmitate.

7. The fuel oil of claim 3 wherein the ester is sorbide dipalmitate.

#### References Cited

#### UNITED STATES PATENTS

|           |         |                    |          |
|-----------|---------|--------------------|----------|
| 2,527,889 | 10/1950 | Moore et al. ----- | 44—66    |
| 2,548,347 | 4/1951  | Caron et al. ----- | 44—66    |
| 2,398,193 | 4/1946  | Sharp -----        | 252—33.4 |
| 2,322,820 | 6/1943  | Brown -----        | 260—333  |

DANIEL E. WYMAN, Primary Examiner

Y. H. SMITH, Assistant Examiner

U.S. Cl. X.R.

44—70; 149—87